

## UNITED STATES PATENT OFFICE

2,383,033

## LUBRICANTS

Elmer Wade Adams, Hammond, Ind., and George W. Flint, Chicago, Ill., assignors to Standard Oil Company, Chicago, Ill., a corporation of Indiana

No Drawing. Application November 2, 1942,  
Serial No. 464,246

9 Claims. (Cl. 252—33)

This invention relates to improvements in small arm lubricants and particularly to lubricants especially adapted for the lubrication and protection of small arms of the type ranging from side arms to machine guns.

In our co-pending application, Serial No. 399,674, filed June 25, 1941, which has matured into Patent No. 2,348,715, of which this is a continuation-in-part, we described therein compositions adapted for the protection of metal surfaces against corrosion, rusting and/or tarnishing. We describe in said application particular petroleum sulfonates which are the active constituents of the slushing compositions described. We have now discovered that these particular petroleum sulfonates when used in combination with certain types of petroleum oils and other addition agents are especially well suited for the lubrication and protection of small size fire arms. Since such materials must be suitable for use under climatic conditions in which wide temperature ranges are encountered they must meet very stringent specifications. In addition to providing the necessary protection against the elements such materials must be capable of providing adequate lubrication at temperatures in excess of 100° F. as well as at temperatures as low as —60 to —70° F.

We have discovered that lubricants meeting these stringent requirements are obtained by compounding certain mineral oils with particular petroleum sulfonates and certain additives consisting essentially of high molecular weight aliphatic oxygen-containing compounds including a substantial proportion of free saturated aliphatic carboxylic acids.

The petroleum sulfonates employed in the present invention are the soaps of sulfonic acids obtained by a particular sulfuric acid treatment of petroleum oils within a definite viscosity range.

Heretofore, it had been the general belief that the soaps of preferentially oil-soluble sulfonic acids obtained by the treatment of petroleum oils with sulfuric acid were of the same type, and therefore were equally effective as inhibitors for the prevention of corrosion and/or the formation of rust. We have now discovered that contrary to the general belief, there is a marked difference in the corrosion inhibiting properties of soaps of preferentially oil-soluble sulfonic acids obtained from oils under various treating conditions. We have discovered that the formation and/or development of tarnish and discoloration upon metal surfaces treated with slushing compounds can be eliminated by employing the soaps of preferen-

tially oil-soluble sulfonic acids derived from a particular sulfuric acid treatment of petroleum oil distillates; namely the soaps of the preferentially oil-soluble sulfonic acids derived by treating distillates of from about 50 seconds to about 1000 seconds or higher, and preferably 200 seconds to 850 seconds to obtain finished oils of from about 200 seconds to about 400 seconds Saybolt Universal viscosity at 100° F. with from about 6 to about 9 pounds, and preferably from about 7 to about 8 pounds of concentrated sulfuric acid, preferably fuming sulfuric acid, per gallon of oil.

The method of obtaining these desirable soaps of preferentially oil-soluble sulfonic acids derived from petroleum oils is illustrated by the following example:

The petroleum oil distillate having Saybolt Universal viscosity at 100° F. of from about 200 seconds to about 850 seconds is treated with from about 7 to about 8 pounds of fuming sulfuric acid per gallon of oil in one-half pound increments or "dumps." After the acid sludge from each one-half pound acid "dump" is settled and withdrawn, the next one-half pound of fuming sulfuric acid is added to the oil. The temperature of the oil before the fuming acid is added thereto is maintained below about 60° F. but due to the heat of reaction upon the addition of the sulfuric acid, the temperature of the oil may rise to from about 90° F. to about 100° F. After the required total amount of fuming sulfuric acid has been added to the oil and the oil freed of acid sludge, the acid treated oil containing oil-soluble sulfonic acids dissolved therein, is neutralized with a solution of sodium hydroxide. The aqueous alkali solution is then separated from the oil solution containing dissolved therein sodium soap of sulfonic acids and the latter then separated from the oil by extraction with alcohol of about 60% strength. The alcohol layer containing dissolved sodium sulfonates is then separated from the oil, and subsequently distilled to recover the alcohol and remove water. The sulfonic soap obtained in this manner contains from about 30% to about 60% sodium sulfonate, from about 30% to about 60% oil, from about 1% to about 10% water, and up to 10% of inorganic salts which may be removed by the procedure hereinafter described.

The above procedure may be modified after the acid sludge is removed from the acid treated oil. The oil containing dissolved sulfonic acids is extracted with about 60% alcohol to remove the sulfonic acids which may then be neutralized with sodium hydroxide and subsequently freed of the alcohol by distillation.

The crude soaps of these preferentially oil-soluble sulfonic acids obtained by the procedure described above may be freed of inorganic salts by purification. This purification is preferably accomplished by dilution of the crude soap with from about  $\frac{1}{2}$  to about 10 parts, preferably 1 to 2 parts of 50% or higher strength alcohol, preferably alcohol of 60 to 70% strength, and allowing the salts to settle while maintaining the mixture within the temperature range of 130 to 175° F., preferably 155 to 165° F. When the salts have settled the supernatant alcohol-soap layer is separated and the alcohol is recovered by conventional distillation procedure.

The soaps of these preferentially oil-soluble sulfonic acids obtained in the manner above described differ from other oil-soluble soaps of sulfonic acids from other fractions such as for example, those obtained by treating petroleum distillates of from about 50 seconds to about 150 seconds Saybolt Universal viscosity at 100° F. with from about 3 pounds to about 4 pounds of fuming sulfuric acid per gallon of oil, and the petroleum sulfonates obtained by treating distillates of from about 80 seconds to about 150 seconds Saybolt Universal viscosity at 100° F. with about 5 pounds of fuming sulfuric acid per gallon of oil. In addition to inhibiting the formation of tarnish and/or discoloration, which other sulfonates do not, the petroleum sulfonates of the present invention differ from other petroleum sulfonates in that the former are substantially less soluble in water than are the latter, although they do show some hydroscopic tendencies.

top of the humidity cabinet. To insure that only moisture of condensation comes in contact with the strips, stainless steel shields are placed above the strips in such a position that no moisture from the shields can drip on the strips. The following petroleum sulfonates were tested under the foregoing conditions:

*Sulfonate I.*—Sulfonates obtained from distillates of 200-850 seconds Saybolt Universal viscosity at 100° F. treated with from about 7 to 20 pounds of fuming sulfuric acid per gallon of distillate, and neutralized with sodium hydroxide. The sulfonate so obtained is that employed in accordance with the present invention.

*Sulfonate II.*—Sulfonates obtained from distillates of from about 50 to about 150 seconds Saybolt Universal viscosity at 100° F. by treating with from 3 to 3½ pounds of fuming sulfuric acid per gallon of distillate, and neutralizing with sodium hydroxide.

*Sulfonate III.*—Sulfonates obtained from distillates of about 80 seconds to about 150 seconds Saybolt Universal viscosity at 100° F. by treating with 5 pounds of fuming sulfuric acid per gallon of distillate, and neutralizing with sodium hydroxide.

Sulfonates II and III are the type of sulfonates heretofore used in slushing compounds. These were found to cause tarnish and discoloration of metal surfaces.

The results obtained in the humidity cabinet tests on naphtha solutions of the foregoing type of petroleum sulfonates are shown in the following table.

TABLE I  
*Humidity cabinet tests of petroleum sodium sulfonates in naphtha solution*

| Petroleum sodium sulfonate | Analysis of sodium sulfonate |             |              |                          | Percent soap used | Duration of test, days | Condition of strips        |
|----------------------------|------------------------------|-------------|--------------|--------------------------|-------------------|------------------------|----------------------------|
|                            | Percent soap                 | Percent oil | Percent salt | Percent H <sub>2</sub> O |                   |                        |                            |
| I.                         | 34.2                         | 58.8        | 4.6          | 6.0                      | 10                | 2                      | No tarnish.                |
|                            | —                            | —           | —            | —                        | 20                | 3                      | Do.                        |
|                            | —                            | —           | —            | —                        | 30                | 5                      | Do.                        |
|                            | —                            | —           | Dry          | —                        | 30                | 3                      | Do.                        |
| II.                        | 46.9                         | 46.2        | 1.8          | 1.6                      | 10                | 2                      | (Severe rust.)<br>Tarnish. |
|                            | —                            | —           | —            | —                        | 20                | 2                      | Severe rust.<br>Tarnish.   |
|                            | —                            | —           | —            | —                        | 30                | 2                      | Severe rust.<br>Tarnish.   |
|                            | —                            | —           | —            | —                        | Dry               | 30                     | Severe rust.<br>Tarnish.   |
| III.                       | 45.7                         | 48.6        | 1.34         | 1.4                      | 30                | 3                      | Severe rust.<br>Tarnish.   |
|                            | —                            | —           | —            | —                        | 30                | 2                      | Severe rust.<br>Tarnish.   |

The effectiveness of the particular petroleum sulfonates used in the present invention in preventing discoloration and/or tarnish of metal surfaces on which it is applied is demonstrated by accelerated tests carried out in a humidity cabinet wherein intermittent periods of heating and cooling are employed while maintaining saturated air conditions within the cabinet. The humidity cabinet which is provided with heating units and thermal regulators for automatic temperature control is maintained on a cycle of 20 hours cooling at 40-45° F. and four hours heating at 100 to 105° F. A water level of 2-3 inches is maintained in the bottom of the cabinet to give approximately saturated conditions at all times. Cold-rolled open hearth steel strips of approximately 1 x 4 inches are coated with the rust preventive material and suspended by glass hooks to a glass rod running across the

00  
65  
70  
75  
80  
85  
90  
95  
100

The foregoing data clearly demonstrate the tarnish forming tendencies of sodium sulfonates II and III and the absence of any tendency of sulfonate I to form tarnish.

Depending upon the severity of the conditions under which the various grades of slushing compounds are to be employed from about 1% to about 40% of the petroleum sulfonates of the present invention are employed in the slushing compounds. While we prefer to employ the sodium soap of such sulfonic acids, other soaps of metals of groups I, II, IV, VI, and VIII of the periodic table may be employed. Thus, for example, we may employ the potassium, calcium, barium, tin, lead, aluminum, chromium, cobalt, and nickel soaps of the sulfonic acids obtained by treating petroleum distillates of from about 50 to about 1000 seconds or higher, and preferably from about 200 seconds to about 850 seconds Say-

bolt Universal viscosity at 100° F. with from about 6 to about 9, and preferably from about 7 to about 8 pounds of fuming sulfuric acid per gallon of distillate.

In accordance with the present invention a petroleum sulfonate of the foregoing type is mixed with a petroleum oil having a Saybolt Universal viscosity at 100° F. within the range of from about 45 seconds to about 70 seconds and a pour test of from about -40° F. to about -70° F.

In addition to the particular type petroleum sulfonate and oil our improved lubricant contains in addition small amounts of a compound which comprises a mixture of aliphatic oxygen-containing compounds of petroleum origin obtained by controlled oxidation of hydrocarbons or mixtures thereof, such as the hydrocarbons occurring in or associated with petroleum oils, in liquid phase at an elevated temperature and under superatmospheric pressure. These aliphatic compounds contain a mixture of substantial quantities of alcohols, ketones, alcohol-ketones, lactones and esters together with some unoxidized hydrocarbons. The method of obtaining these oxygen-containing aliphatic compounds and the compositions thereof are described in United States Patents 1,690,768, 1,690,769 and 1,863,004 and others issued to A. W. Burwell. Products of the type described in these patents are marketed under the trade name of "Alox" compounds; compounds marketed as "Alox 152," "Alox 350" and "Alox 600" are well suited for this purpose. For the purpose of identifying these compounds they will be referred to hereinafter in this specification and the appended claims as "petroleum oxidation products."

For the purpose of lubricating and protecting fire arms of the type described compositions falling within the following approximate ranges can be employed:

|                                          | Per cent |
|------------------------------------------|----------|
| Mineral oil <sup>1</sup>                 | 70-90    |
| Sodium sulfonate <sup>2</sup> (oil free) | 2-10     |
| Petroleum oxidation products             | 1/2-6    |

<sup>1</sup> Saybolt Universal viscosity at 100° F. 50-55 seconds—pour point about -60° F.

<sup>2</sup> Obtained by treating distillates of from about 200 seconds to about 850 seconds Saybolt Universal viscosity at 100° F. with 7-8 pounds of fuming sulfuric acid and neutralizing the sodium hydroxide.

The "petroleum oxidation products" which we have found well suited for use in the above compositions are products marketed as "Alox 152," "Alox 600" and "Alox 350." These may be used in amounts ranging from 0.5% to 6.0% respectively or collectively in the finished oil.

A product which has been found particularly well suited for the lubrication and protection of small fire arms is one having the following approximate composition:

|                                                                          | Per cent |
|--------------------------------------------------------------------------|----------|
| Mineral oil <sup>1</sup>                                                 | 82       |
| Oil-containing sodium sulfonate <sup>2</sup> (oil-free approximately 5%) | 14       |
| Petroleum oxidation product <sup>3</sup>                                 | 4        |

<sup>1</sup> Saybolt Universal viscosity at 100° F. 50-55 seconds—pour point about -60° F.

<sup>2</sup> Obtained by treating distillates of from about 200 seconds to about 850 seconds Saybolt Universal viscosity at 100° F. with 7-8 pounds of fuming sulfuric acid and neutralizing the sodium hydroxide.

<sup>3</sup> Preferably the product marketed as "Alox 600" or the product marketed as "Alox 152."

Another effective composition is one having approximately the same compositions as the above except that the "petroleum oxidation product" is

a blend of 2% of the product marketed as "Alox 600" and 2% of the product marketed as "Alox 350."

Still another effective composition is one having approximately the following composition:

|                                          | Per cent |
|------------------------------------------|----------|
| Mineral oil <sup>1</sup>                 | 88-94    |
| Sodium sulfonate <sup>2</sup> (oil free) | 6.0-12   |

<sup>1</sup> Saybolt Universal viscosity at 100° F. approximately 45-70 seconds; pour point approximately -40° F.-70° F.

<sup>2</sup> Obtained by treating distillates of from about 200 seconds to about 850 seconds Saybolt Universal viscosity at 100° F. with 7-8 pounds of fuming sulfuric acid and neutralizing the sodium hydroxide.

Products of the foregoing compositions have been found to effectively lubricate small size fire arms at temperatures as low as -70° F. and have provided complete corrosion protection for a period of 200 hours in an atmosphere maintained at 100° F. and 100% humidity.

While we have described the present invention in connection with the lubrication and protection of fire arms it is to be understood that the same is not limited thereto. Obviously our improved products are equally well adapted for the lubrication and protection of other metal articles, such as highly finished metal articles, for example, fishing reels, cutlery, sewing machines, and the like.

Although we have described the invention in connection with certain specific embodiments thereof it is understood that these are by way of illustration only and not by way of limitation.

We claim:

1. A composition of matter comprising a major proportion of a mineral oil having a Saybolt Universal viscosity at 100° F. within the range of about 45 seconds to about 70 seconds, from about 1% to about 40% of a soap of preferentially oil-soluble sulfonic acids obtained by treating a petroleum distillate having a Saybolt Universal viscosity at 100° F. within the range of about 50 seconds to about 1000 seconds with from about 6 pounds to about 9 pounds of concentrated sulfuric acid per gallon of distillate, and from about 0.5% to about 6% of a mixture of saturated aliphatic oxygen-containing compounds including alkyl ester, lactones, ketones, alcohols and alcohol-ketones, said saturated aliphatic oxygen-containing compounds being obtained by the partial oxidation of petroleum hydrocarbons.

2. A composition of matter comprising a major proportion of a mineral oil having a Saybolt Universal viscosity at 100° F. of from about 45 seconds to about 70 seconds and a pour point of at least about -40° F., from about 1% to about 40% of a metal soap of preferentially oil-soluble sulfonic acids obtained by treating a petroleum distillate having a Saybolt Universal viscosity at 100° F. of from about 50 seconds to about 1000 seconds with from about 6 pounds to about 9 pounds of concentrated fuming sulfuric acid per gallon of distillate, and from about 0.5% to about 6% of a mixture of saturated aliphatic oxygen-containing compounds including alkyl esters, lactones, ketones, alcohols and alcohol-ketones, obtained by the partial oxidation of petroleum hydrocarbons.

3. A composition of matter as described in claim 2 in which the metal soap is sodium soap.

4. A composition of matter as described in claim 2 in which the metal soap is calcium soap.

5. A composition of matter as described in

claim 2 in which the metal soap is aluminum soap.

6. A mineral oil composition having a pour point of at least about -40° F. and adapted for the lubrication and protection of metal articles comprising a major proportion of a petroleum oil having a Saybolt Universal viscosity at 100° F. of from about 45 seconds to about 70 seconds and a pour point of at least about -40° F., from about 1% to about 40% of an alkali metal soap of preferentially oil-soluble sulfonic acids obtained by treating a petroleum distillate having a Saybolt Universal viscosity at 100° F. of from about 200 seconds to about 850 seconds with from about 7 to about 8 pounds of fuming sulfuric acid per gallon of distillate, and from about 0.5% to about 6% of a mixture of saturated aliphatic oxygen-containing compounds including alkyl esters, lactones, ketones and alcohols, said oxygen-containing compounds being obtained by the partial oxidation of petroleum hydrocarbons.

7. A composition of matter comprising about 70% to about 90% mineral oil having a Saybolt Universal viscosity at 100° F. within the range of about 45 seconds to about 70 seconds, about 2% to 10% of a soap of preferentially oil-soluble sulfonic acids obtained by treating a petroleum distillate having a Saybolt Universal viscosity at 100° F. within the range of about 50 seconds to about 1000 seconds with from about 6 pounds to about 9 pounds of concentrated sulfuric acid per gallon of distillate, and about 0.5% to 6% of a mixture of saturated aliphatic oxygen-containing compounds obtained by the partial oxidation of petroleum hydrocarbons.

8. A composition of matter comprising about

70% to 90% of a mineral oil having a Saybolt Universal viscosity at 100° F. of from about 45 seconds to about 70 seconds and a pour point of at least about -40° F., about 2% to 10% of a metal soap of preferentially oil-soluble sulfonic acids obtained by treating a petroleum distillate having a Saybolt Universal viscosity at 100° F. of from about 50 seconds to about 1000 seconds with from about 6 pounds to about 9 pounds of concentrated fuming sulfuric acid per gallon of distillate, and about 0.5% to 6% of a mixture of saturated aliphatic oxygen-containing compounds including alkyl esters, lactones, ketones, alcohols and alcohol-ketones, obtained by the partial oxidation of petroleum hydrocarbons.

9. A fire-arm lubricant and coating composition adapted for service at temperatures as low as at least -40° F. comprising about 70% to 90% of a mineral oil having a Saybolt Universal viscosity at 100° F. of from about 45 seconds to about 70 seconds and a pour point of at least about -40° F., about 2% to 10% of an alkali metal soap of preferentially oil-soluble sulfonic acids obtained by treating a petroleum distillate having a Saybolt Universal viscosity at 100° F. of from about 50 seconds to about 1000 seconds with from about 6 pounds to about 9 pounds of concentrated fuming sulfuric acid per gallon of distillate, and about 0.5% to 6% of a mixture of saturated aliphatic oxygen-containing compounds including alkyl esters, lactones, ketones, alcohols and alcohol-ketones, obtained by the partial oxidation of petroleum hydrocarbons.